

## UNITED STATES PATENT OFFICE

2,365,833

PROCESS OF INCORPORATING POLY-  
CHLOROPHENOLS IN FIBERBOARD

Henry L. Morrill, Clayton, and John D. Fleming,  
St. Louis, Mo., assignors to Monsanto Chemical  
Company, St. Louis, Mo., a corporation of Dela-  
ware

No Drawing. Application September 5, 1939,  
Serial No. 293,428

2 Claims. (Cl. 92—21)

The present invention relates to fiber board, particularly fiber boards which are made from mechanically disintegrated wood, for example, from fibers resulting from the explosive disintegration process, and relates specifically to methods of incorporating toxic polychlorophenols such as pentachlorophenol into such boards.

The principal object of the present invention is to provide a method of incorporating polychlorophenols uniformly in fiber boards.

Wood can be disintegrated to fibers suitable for felting and forming boards by various methods. These methods can be classified generally as chemical disintegration processes or mechanical disintegration processes. In chemical disintegration processes, wood, preferably in the form of chips or in a similar comminuted form, is treated with chemicals such as sodium sulfite or sodium hydroxide and the resulting fibers are refined, mixed with binding ingredients, if necessary, formed into felts and these felts are then dried and molded into boards. Boards are formed in the mechanical disintegration processes in much the same general manner except that the wood chips are disintegrated into fibers by grinding, explosion, or similar mechanical disintegration methods. The present invention relates particularly to boards and the process of making them from fibers produced by the explosion method of mechanical disintegration.

The explosion method of mechanically disintegrating wood and forming boards from the fibers thus produced has been described by W. H. Mason in Paper Trade Journal, 1927, vol. 84, No. 8, pages 131-136 and by Robert M. Boehm in Industrial and Engineering Chemistry, 1930, vol. 22, pages 493-497. The commercial product is known as Masonite and appears in several forms, differing principally in density as a result of the molding conditions used in the final forming operation. In the explosion process the wood to be disintegrated is prepared in the form of chips. The types of wood to be used may be varied, since practically no species of wood is unsuitable for manufacture of board by the explosion process. Soft woods such as spruce, as well as hard woods are usable. However, since the strength of the board is dependent to some extent upon the fibrous structure as well as the proportion and nature of certain of the wood constituents, long-leaf pine, southern gum and mixtures of the two are preferred because of their availability and desirable characteristics. The wood chips are then placed in metal autoclaves, which are called guns, provided at the

bottom with quick-opening hydraulic valves for the release of the loads and with inlets for steam at the top. The load of wood chips in the guns is then subjected to steam at a pressure of about 5 350 pounds per square inch, bringing the chips to a temperature of about 375° F. (190° C.), and is maintained at this temperature for about 30 to 40 seconds. The pressure is then increased to about 1000 pounds per square inch and maintained thereat for about 5 seconds, the temperature reaching about 540° F. (282° C.). While at this high steam pressure the hydraulic discharge valve is opened and the chips pass through a small port in the bottom of the gun 10 where they explode immediately. In the explosion the chip is ruptured as a result of the high internal pressure within the chip and a mass of long fiber bundles is produced. The exploded fibers are then separated from the steam, pass to a storage chest, and are subsequently refined, that is, subjected to mechanical grinding to break down the bundles slightly, screened to remove coarse particles and mechanically treated to obtain a suspension of fibers of the desired 15 consistency and uniformity. The fibers may be subjected to one or more refining operations of this type. The stock then passes to a stock chest. The fiber may be treated with an emulsion of paraffin or a similar substance to impart to 20 the board a degree of water-repellency. Such sizing operations may, however, be omitted. The fiber suspension from one or more stock chests passes through a head box and is then felted on a machine similar to a Fourdrinier to produce a 25 wet lap of fibers about 2 inches thick. The white water from this operation may be clarified and recirculated. This felting machine is provided with suction boxes and press rolls over which the felt passes and where it is reduced to 30 about  $\frac{3}{4}$  inch thickness and is left with a content of about 65 per cent water. The lap is then cut in suitable sizes, and subsequently dried in heated presses. The pressed board may be later rehumidified or seasoned to diminish its 35 tendency to warp or expand.

Heretofore for incorporating polychlorophenols such as trichlorophenols, tetrachlorophenols, and pentachlorophenol into fiber boards a number of methods have been tried. To beat up the polychlorophenol in powdered form with the pulp is 40 unsatisfactory because of the difficulty of grinding the polychlorophenol to a sufficiently fine form to obtain uniform and intimate distribution of the compound in the fiber suspension. Another method 45 consists in incorporating the polychlorophenol

as a sodium salt in the pulp or fiber suspension and thereafter precipitating the fibers together with the size, which is usually an alkaline solution of rosin, by the use of alum, for example, in the beater. Much of the polychlorophenol is retained in the white water and this is an economic disadvantage militating against the general use of the process. To overcome this loss in the white water, processes have been described for precipitating the polychlorophenol from its sodium salt in the presence of the pulp in the form of a less soluble metal salt, such as a zinc salt. The cost of the metal precipitating salt is a great obstacle to the use of this process inasmuch as the additional protection afforded by the metal present in the resulting polychlorophenol compound does not add substantially to the protective value of the polychlorophenol. Furthermore, the common metal salts of pentachlorophenol, the polychlorophenol with the lowest solubility in water, are actually more soluble in water than the free phenol. Such is the case with the zinc, calcium, barium and copper salts of pentachlorophenol. The method of precipitating the polychlorophenol from its sodium salt in the presence of the pulp or fiber by means of an acid, as heretofore applied to various pulps and fiber suspensions, leaves a great proportion of the polychlorophenol in the white water.

It has now been discovered that polychlorophenols can be incorporated uniformly into fiber boards made from exploded fibers during the manufacture of board therefrom by adding the polychlorophenol as the sodium or other water-soluble salt to the exploded fibers contained in the storage chest or stock chest or at the head box in the process briefly outlined hereinbefore for producing fiber board by the explosive disintegration method. This incorporation also results with but a small fraction of the expected losses in the white water and by modifying the process as herein described even these small losses can be drastically reduced.

The solubility of pentachlorophenol in water, in percentages by weight at various temperatures, is given in the table hereinbelow:

| Temperature, °C. | Solubility of pentachlorophenol, percent by weight |
|------------------|----------------------------------------------------|
| 0                | 0.0005                                             |
| 27               | 0.0018                                             |
| 50               | 0.0035                                             |
| 62               | 0.0058                                             |
| 70               | 0.0085                                             |

The solubility of pentachlorophenol in aqueous acetic acid having a pH of 2.0 is about 0.0040% at 40° C., compared to 0.0025% in distilled water at the same temperature.

When it is considered that the fiber stock in the production of boards is maintained at a temperature of 160° F. (71° C.) during the refining operations and is not substantially cooler during the felting, and it is known that the fiber stock contains acids such as tannic, acetic and formic acids, it was unexpected that the white water losses would not be excessive and much higher than would result from the use of a cold fiber stock suspended in water free from excess acid. Yet such was the discovery that was made when the process was adopted in practice.

It was discovered that the fibers resulting from the explosion process actually removed penta-

chlorophenol from an aqueous solution of pentachlorophenol. By stirring up 100 grams of exploded fibers with about 5,000 grams of a dilute aqueous solution of pentachlorophenol the concentration of the solution dropped from an original concentration of about 23 parts per million to about 2.6 parts per million of pentachlorophenol. This indicates that the fiber takes up about 0.1% pentachlorophenol directly from an aqueous solution by adsorption or a similar phenomenon. Ordinarily it would be expected that the fibers would take up the solution more or less by absorption or entrainment and no reduction of the concentration of the solution would result. The advantages resulting from operating according to the method of this invention are in part attributable to the characteristics of the fibers obtained by the explosive disintegration of wood and partly to the complex composition of the white water and the nature of its reaction upon the salt of the polychlorophenols.

In the practice of the present invention the process of producing boards by the explosive disintegration of wood is not substantially modified. The wood is disintegrated in the usual manner, the stock is felted in the conventional manner and the water is removed from the felts and the board is pressed between heated platens as heretofore. However, after the fiber is exploded a water-soluble salt of the polychlorophenol is added to the fiber stock in the storage chest, stock chest or head box, that is, the salt is added before or after refining. The proportion of salt of the polychlorophenol, for example, sodium pentachlorophenate, which is added is such that a sufficient concentration of the polychlorophenol is left in the board. Generally pentachlorophenol in an amount equivalent to 1% by weight of technical sodium pentachlorophenate (which has an assay of about 90%  $NaOC_6Cl_5$ ) in the finished board is ample. The quantity of sodium pentachlorophenate to be added can be approximated by taking into account the greatest amount of water present in the stock at any point in the process (roughly, the stock will contain from 1 to 2% of fiber and 98 to 99% water) and the solubility of the pentachlorophenol in the water at the particular temperature or at the highest temperature which will be encountered in the process. Since the apparent solubility of the pentachlorophenol in the water in the presence of the fiber will be less than that expected, it will be necessary to add an excess of sodium pentachlorophenate corresponding only to this apparent solubility in order to saturate the water with pentachlorophenol. Inasmuch as reuse of the white water is contemplated and such white water is already substantially saturated with pentachlorophenol, that is, saturated with respect to that proportion of pentachlorophenol which can be retained in solution in the presence of the fiber, the quantity of sodium pentachlorophenol to be added after the water system is saturated will be simply that required to provide the desired proportion in the board. When polychlorophenols other than pentachlorophenol are to be used, slight variations influenced by the different solubility of the polychlorophenol, the difference in absorption on the fibers and similar factors must be considered. As an example, to provide a board containing pentachlorophenol in an amount equivalent to 1% technical (90%) sodium pentachlorophenate, 1.2 pounds of 90% sodium pentachlorophenate in the form of an aqueous 14% solution are added to 120 pounds of

dry exploded fiber (calculated on the average yield from the wood chips which were charged into the gun) in customary operations, after the water used in the system has become saturated by recirculation.

After the water-soluble salt of the polychlorophenol has been added to the fiber stock at one of the indicated points in the process, immediate precipitation occurs and the fibers become coated with and entangle or entrain the polychlorophenol precipitate as well as take up a large proportion of the polychlorophenol that is not precipitated. This precipitation of polychlorophenol results from the acidity of the fiber stock which has a natural acidity corresponding to a pH value of approximately 4.5. Contrary to expectations, since addition of sodium pentachlorophenate, for example, to an aqueous solution of acid reduces the initial acidity, there is no substantial reduction of acidity or increase in pH value of the white water associated with the fiber stock on adding small percentages of sodium pentachlorophenate thereto. The natural constituents of the white water influence the character of precipitate and the character of the precipitate has much to do with its retention on and in the fibrous structure.

The process of producing board from the stock to which the water-soluble salt of the polychlorophenol has been added is then conducted in the usual manner. This consists briefly in preparing the felt on the felting machine and subsequently pressing the felt between heated platens. The white water recovered from the felting operation is then clarified and reused in preparing the fiber stock. Heretofore, in the molding of felts containing polychlorophenols, considerable difficulty has been experienced in the polychlorophenol "bleeding" or concentrating at the surface and being lost by volatilization after removal from the press. No such difficulty has been experienced with felts prepared by the improved process of this invention.

The sizing of the fibers to impart water-repellency to the board may be conducted in the conventional manner, that is, by adding an emulsion of paraffin wax to the fiber suspension in the stock chest. With regard to protective action of the polychlorophenol in the finished board, there is substantially no difference between adding the polychlorophenol before or after the paraffin wax emulsion has been added to the fiber suspension.

The process described herein may be used for

incorporating such polychlorophenols as the various isomeric trichlorophenols and tetrachlorophenols and pentachlorophenol into the board. The water-soluble salts which may be used include those of the alkali metals. The sodium salts are the most readily obtained commercially and the cheapest, hence are preferred. The 90% technical sodium pentachlorophenate which is referred to herein is the commercially available material that assays 90%  $\text{NaOC}_6\text{Cl}_5$ , the other constituents of which include water and small proportions of neutral salts and sodium salts of other phenolic bodies.

10 Fiber board resulting from the process of the invention containing uniformly distributed therethrough from about 1% to 5% or more of a polychlorophenol is resistant to attack by mildew, fungi, insects, particularly termites, and similar pests.

15 20 Inasmuch as the foregoing description comprises preferred embodiments of the invention it is to be understood that the invention is not restricted thereto, and that variations and modifications may be made therein without departing substantially from its scope, as defined in the appended claims.

We claim:

1. The process of producing insect and mildew-proofed fiber board having uniformly distributed 30 therethrough on the fibers thereof a polychlorophenol selected from the group consisting of trichlorophenol, tetrachlorophenol and pentachlorophenol comprising explosively disintegrating wood, preparing a fiber stock by addition of water 35 to the fibers and the acidic aqueous liquor resulting from said explosive disintegration, adding to said fiber stock a water-soluble salt of a polychlorophenol selected from the group consisting of trichlorophenol, tetrachlorophenol and 40 pentachlorophenol, whereby the said polychlorophenol is precipitated by the water-soluble constituents contained in the aqueous liquor resulting from the explosive disintegration of the wood, felting the resulting stock, and thereafter molding 45 said felts into boards, and reusing a substantial portion of the acidic white water recovered in said felting for subsequent stock preparation.

2. The process as defined in claim 1 and further characterized in that the water-soluble salt of a polychlorophenol is sodium pentachlorophenate.

HENRY L. MORRILL.  
JOHN D. FLEMING.